

# UNITED STATES PATENT OFFICE.

SABURO KASHITANI, OF IMAMIYA MACHI, JAPAN.

## PROCESS OF TREATING COTTON AND COTTON MANUFACTURES.

1,360,224.

Specification of Letters Patent. Patented Nov. 23, 1920.

No Drawing.

Application filed December 10, 1918. Serial No. 266,122.

To all whom it may concern:

Be it known that I, SABURO KASHITANI, a subject of the Emperor of Japan, and resident of 823 Motokizu, Imamiya Machi,

5 Nishinari Gun, Osaka Fu, Empire of Japan, have invented new and useful Improvements in Processes of Treating Cotton and Cotton Manufactures, of which the following is a specification.

10 This invention has reference to improvements in processes of treating cotton or cotton manufactures to remove fine surface hairs or fibers, impart luster thereto and produce a soft, fine textile capable of being 15 dyed and colored and resembling in appearance a superior quality of hemp.

In general terms the present process contemplates treating cotton and cotton manufactures with concentrated sulfuric acid to 20 render the same amyloid, removing fine hairs or fibers from the surface of the cotton yarn by utilization of the adhesive qualities of the amyloid formed thereon, neutralizing the sulfuric acid and imparting a 25 desirable hardness and luster thereto by subjecting the same to a bath of caustic soda solution, and treating the same with a water solution of borax to prevent damage thereto attributable to the action of acid and to 30 render the same fireproof, and producing a pleasing softness, and texture by treatment of the cotton or cotton manufactures with a solution of glycerin.

It is conceded that separate and distinct 35 processes have heretofore been known for treating textiles with concentrated sulfuric acid, neutralizing acid by means of caustic soda and rendering fabric fireproof by submersion in a water solution of borax as 40 suggested by Doeberciner and Gay Lussac, but the method of removing the amyloid and consequently fine hairs and fibers from cotton and cotton manufactures and treating the same to produce a textile of the 45 character disclosed hereafter is believed to be a great improvement in the art to which this invention appertains.

Furthermore the present process chemically changes the original textile instead of 50 subjecting the same to a mere aggregation of mechanical operations to produce the desired result, thus facilitating and expediting

the manufacture of the product and greatly reducing overhead cost as represented by an imposing outlay of complicated machinery 55 and many skilled operators.

For the purpose of illustrating the application of the present process, there is described hereinafter in detail one method which is at present preferred, since the same 60 has been found in practice to give satisfactory and reliable results, although it is to be understood that the various steps of which the process consists can be differently arranged and organized, and such chemicals 65 as have alternatives, can be used provided such departures from the precise disclosure fall within the spirit of the invention and the scope of the claims as appended hereunto.

In order that the process will be clearly defined in the mind of one skilled in the art to which the invention appertains the following major steps or operations are outlined.

1. The cotton or cotton manufacture is subjected to a bath in 52 degrees Baumé to 60 degrees Baumé concentrated sulfuric acid and allowed to remain therein from one to fifteen minutes according to the degrees of 80 refining and the size of the yarn, whereupon it is removed from the bath and washed in water to remove as much of the acid as is possible.

2. The fabric or yarn, as the case may be, 85 is then stretched and beaten to open or distend the meshes or fibers to remove the amyloid therefrom and as the amyloid is adhesive the fine hairs or fibers will also be removed from surface thereof.

90 3. The whole is then dipped in an 8 degrees Baumé to 15 degrees Baumé solution of caustic soda for ten or twenty minutes to neutralize the action and prevent the discoloring effect of the sulfuric acid, to 95 impart suitable hardness thereto, and to produce a certain luster on the textile, whereupon the same is thoroughly washed in water.

4. The fabric or yarn is then treated with 100 a 3 per cent. water solution of borax to absolutely neutralize the free acid and to render the same fireproof.

5. The same is dipped in a 5 per cent.

solution of glycerin to render it soft and pleasing to the skin.

The above steps or operations having been completed the cotton or cotton manufacture 5 possesses a desirable toughness and luster and resembles in softness and texture a very superior quality of hemp and may be readily dyed or in the case of yarn may be woven or knitted into cloth or other fabrics.

10 Furthermore when it is desired to render the same waterproof it may be treated with aluminum acetate or other chemical which will in no way decrease its utility or appearance.

15 In connection with the sulfuric acid bath as described in the first step or operation it is pointed out that some discretion must be used as to the strength of the solution and the duration of the bath, as a high concentration of acid or a too lengthy bath may convert the whole yarn or fabric to amyloid, while the desired result is similar to that which is obtained by a mechanical process such as gassing the yarn or fabric. Furthermore the proper treatment with sulfuric acid effects a very slight chemical change in 25 the cotton other than amyloidization which makes it possible to remove the amyloid and fine hairs and fibers easily and with the desired results.

30 In order to more clearly define the second step or operation the following simple experiment is suggested: Treat a piece of cotton goods with sulfuric acid as above described and thoroughly wash the same in water, whereupon stretch the same with the hands until the meshes are opened or enlarged thus loosening and permitting the amyloid between the strands to be removed 35 by beating or shaking along with the fine hairs and fibers. In the case of yarn or strands of cotton the desired result may also be obtained by combing. Furthermore it is stated that when cotton has been so treated 40 the fibers of the cotton yarn contract and have the appearance of being double-folded or tightened, while similar treatment of cotton manufactures or fabrics such as knitted goods or the like enlarges the meshes to improve ventilation and to produce when handled a pleasant sound.

45 Relative to the application of the fifth step or operation as above outlined, namely the glycerin bath, it is stated that alternatives for the solution of glycerin may be used if desired and these have been found by experiment to comprise any one of the following:—calcium-chlorid solution, glucose solution or soap suds.

50 Having described the process and its product with such attention to detail as will

thoroughly acquaint one skilled in the art with its operation and advantages, I claim—

The hereinbefore described process of treating cotton or cotton manufactures consisting in subjecting the same to an acid bath, distention and agitation, a neutralizing bath for the acid, a further neutralizing bath for the acid and to substantially fireproof the same, and dipping the same into a bath to render the resulting product soft and pleasing to the touch.

65 The hereinbefore described process of treating cotton or cotton manufactures consisting in subjecting the same successively to an acid bath, to mechanical distention and agitation, to a neutralizing bath for the acid, to a further neutralizing bath for the acid and to render the same substantially fireproof, and dipping the same into a glycerin 70 bath to render it soft and pleasing to the touch.

75 The hereinbefore described process of treating cotton or cotton manufactures consisting in subjecting the same successively to a sulfuric acid bath, to mechanical distention and agitation, to a caustic soda bath, to a bath in a solution of borax and to a bath in a solution of glycerin for the purposes set forth.

80 The hereinbefore described process of treating cotton or cotton manufactures consisting in subjecting the same successively to a bath in 32 degrees Baumé to 60 degrees Baumé concentrated sulfuric acid, to mechanical distention and agitation, to a bath in 3 degrees Baumé to 15 degrees Baumé solution of caustic soda, to a bath in a 3 degrees Baumé solution of borax and to a bath in a 3 per cent. solution of glycerin for the 85 purposes set forth.

90 The hereinbefore described process of

treating cotton or cotton manufactures consisting in subjecting the same successively to a

95 bath in 32 degrees Baumé to 60 degrees Baumé concentrated sulfuric acid, to mechanical distention and agitation, to a bath in 3 degrees Baumé to 15 degrees Baumé solution of caustic soda, to a bath in a 3 degrees Baumé solution of borax and to a bath in a 3 per cent. solution of glycerin for the 100 purposes set forth.

105 The hereinbefore described process of treating cotton or cotton manufactures consisting in subjecting the same successively to submersion from one to ten minutes in a bath of 32 degrees Baumé to 60 degrees Baumé concentrated sulfuric acid to render the same amyloid, mechanically distending, agitating and beating the same to remove the amyloid and the fine hairs and fibers, a bath of ten to twenty minutes duration in an 110

degree Baumé to 15 degrees Baumé solution of caustic soda to neutralize the sulfuric acid, a treatment with a 3 per cent. aqueous solution of borax to complete neutralization and render the same fire resisting, and finally dipping the product in a 5 per cent. solution of glycerin to render it soft and pleasing to the touch.

115 A testimony whereof I affix my signature 120 hereto.

ABURO KASHITANI.